



US009951400B1

(12) **United States Patent**  
**McDevitt et al.**

(10) **Patent No.:** **US 9,951,400 B1**  
(45) **Date of Patent:** **Apr. 24, 2018**

(54) **WROUGHT MACHINABLE BRASS ALLOY**

(71) Applicant: **Chase Brass and Copper Company, LLC**, Montpelier, OH (US)

(72) Inventors: **David Dean McDevitt**, Angola, IN (US); **Charles Lawrence Muller**, Wauseon, OH (US)

(73) Assignee: **CHASE BRASS AND COPPER COMPANY, LLC**, Montpelier, OH (US)

(\*) Notice: Subject to any disclaimer, the term of this patent is extended or adjusted under 35 U.S.C. 154(b) by 162 days.

(21) Appl. No.: **14/817,191**

(22) Filed: **Aug. 3, 2015**

**Related U.S. Application Data**

(63) Continuation of application No. 14/493,164, filed on Sep. 22, 2014, now abandoned.

(60) Provisional application No. 61/937,464, filed on Feb. 7, 2014.

(51) **Int. Cl.**  
**C22C 9/04** (2006.01)

(52) **U.S. Cl.**  
CPC ..... **C22C 9/04** (2013.01)

(58) **Field of Classification Search**  
CPC ..... B21C 23/002; C22C 9/04; C22F 1/08

USPC ..... 420/479  
See application file for complete search history.

(56) **References Cited**

**U.S. PATENT DOCUMENTS**

|                   |        |             |       |           |
|-------------------|--------|-------------|-------|-----------|
| 6,413,330 B1      | 7/2002 | Oishi       | ..... | 148/434   |
| 7,056,396 B2 *    | 6/2006 | Oishi       | ..... | C22C 9/04 |
|                   |        |             |       | 148/434   |
| 7,883,589 B2      | 2/2011 | Oishi       | ..... | 148/434   |
| 7,909,946 B2      | 3/2011 | Oishi       | ..... | 148/434   |
| 2013/0177472 A1   | 7/2013 | Dahl et al. | ..... | 420/477   |
| 2014/0112821 A1 * | 4/2014 | Yamamoto    | ..... | C22C 9/04 |
|                   |        |             |       | 420/475   |

**FOREIGN PATENT DOCUMENTS**

|    |             |        |       |           |
|----|-------------|--------|-------|-----------|
| JP | 2004-183056 | 7/2004 | ..... | C22C 9/04 |
| WO | 2013/047991 | 4/2013 | ..... | C22C 9/04 |

\* cited by examiner

*Primary Examiner* — Jie Yang

(74) *Attorney, Agent, or Firm* — Harness, Dickey & Pierce, P.L.C.

(57) **ABSTRACT**

A wrought machinable low copper, silicon, zinc alloy having a copper content between about 66 weight percent and about 70 weight percent and wherein the silicon content is between about 1.3 weight percent and about 2.0 weight percent.

**6 Claims, 29 Drawing Sheets**







Fig. 1A



Fig. 2

Figure 3 - ISO 6509 Corrosion Depth (μm)



Figure 4 - Elongation (%)





Fig. 5



Fig. 6



**Fig. 7**



Fig. 8



Fig. 9



Fig. 10



Fig. 11



Fig. 12



Fig. 13



Fig. 14



Fig. 15



Fig. 16



Fig. 17



Fig. 18



Fig. 19



Fig. 20



Fig. 21



Fig. 22



Fig. 23



Fig. 24



Fig. 25



Fig. 26



Fig. 27



Fig. 28

## WROUGHT MACHINABLE BRASS ALLOY

## CROSS-REFERENCE TO RELATED APPLICATIONS

This application is a continuation application which claims priority to U.S. application Ser. No. 14/493,164 filed on Sep. 22, 2014, which claims priority to U.S. Provisional Application Ser. No. 61/937,464 filed on Feb. 7, 2014, the disclosures of which are incorporated by reference in their entirety.

## FIELD

The present disclosure relates to wrought copper alloys, and in particular to low copper, machinable brass alloys, with low or no lead.

## BACKGROUND

This section provides background information related to the present disclosure which is not necessarily prior art.

Lead is a common ingredient in copper alloys to improve their machinability. Typical lead contents in machinable brass alloys range from about 1 to about 6 percent (by weight). Because of their excellent machinability, these lead-containing copper alloys have been an important basic material for a variety of articles such as water faucets, and supply/drainage metal fittings and valves.

However, the application of these lead-containing alloys has been limited in recent years, because the lead contained therein is believed to be an environmental pollutant harmful to humans. One aspect is the lead contained in metallic vapor that is generated in the manufacturing and processing of these alloys at high temperatures, such as in melting and casting operations. Another aspect is the concern that lead contained in water system metal fittings, valves, and other components made of those alloys will dissolve out into the water supply.

For these and other reasons, many countries have been reducing the permissible levels of lead in plumbing fixtures. While there are a number of copper alloys that can be used, most of these alloys are very difficult or expensive to machine into satisfactory plumbing parts. Various attempts have been made to provide copper alloys with improved machinability for these applications. One good example of such an alloy is C87850, which has a nominal composition of 74-78 weight percent copper, up to 0.1 weight percent antimony, up to 0.1 weight percent iron, up to 0.09 weight percent lead, up to 0.1 weight percent manganese, up to 0.2 weight percent nickel, between 0.05 and 0.2 weight percent phosphorus, between 2.7 and 3.4 weight percent silicon, up to 0.3 weight percent tin, and the balance zinc. Several patents cover C87850 and related alloys, including U.S. Pat. Nos. 6,413,330, 7,056,396, and 7,883,589. These patents teach that for copper contents <70 weight percent "the addition of less than 2.0 percent, by weight, of silicon cannot form a gamma phase sufficient to provide industrially satisfactory machinability." They further teach that a minimum copper content of about 69 weight percent is needed to provide a satisfactory alloy.

While these alloys provide excellent properties for plumbing and other applications, are readily machinable, and they include little to no lead, these alloys can be relatively expensive to manufacture.

## SUMMARY

This section provides a general summary of the disclosure, and is not a comprehensive disclosure of its full scope or all of its features.

Alloys of the present invention likewise provide excellent properties for plumbing and other applications, are readily machinable, and they likewise include little to no lead. However, unlike the prior art machinable copper alloys with little to no lead, these alloys have reduced copper and silicon contents and are therefore less expensive than the well-known prior art machinable copper alloys which contain more copper and less zinc.

Generally embodiments of this invention provide wrought products of a machinable low lead, low copper, silicon, zinc alloy. In a preferred embodiment the alloy comprises between about 66 and about 70 weight percent copper, and the silicon content is between about 1.3 weight percent and about 2.0 weight percent, and the balance comprises primarily zinc, and unavoidable impurities. In some preferred embodiments the alloy comprises between about 66 and about 69 weight percent copper, and the silicon content is between about 1.5 weight percent and about 2.0 weight percent.

In a further preferred embodiment the Si content further satisfies the relationship:  $0.167\text{Cu}-9.28>\text{Si}>0.132\text{Cu}-7.66$ .

Some embodiments can contain additional elements, including up to about 0.15 weight percent phosphorus, up to about 0.5 weight percent iron, up to about 1.2 weight percent tin, up to about 2.5 weight percent aluminum, up to about 0.25 weight percent nickel, up to about 0.25 weight percent cobalt, up to about 0.25 weight percent manganese, up to about 0.15 weight percent arsenic, up to about 0.15 weight percent antimony, up to about 0.25 weight percent bismuth, up to about 0.25 weight percent selenium, and up to 0.25 weight percent sulfur.

In some embodiments there is only one of tin and aluminum. In other embodiments, there is only a nominal amount of both tin and aluminum.

The alloy is preferably corrosion resistant, and preferably has corrosion penetration  $\leq 200\text{ }\mu\text{m}$  when tested according to ISO 6509 Protocol, and more preferably  $\leq 100\text{ }\mu\text{m}$  tested according to ISO 6509 Protocol.

The alloy preferably has a tensile strength of at least about 55 ksi as determined according to ASTM E8, and more preferably at least about 65 ksi as determined according to ASTM E8. The alloy preferably has a yield strength of at least 20 ksi as determined according to ASTM E8, and more preferably at least 30 ksi as determined according to ASTM E8. The alloy preferably has a surface hardness (Rockwell B) of at least 55 as determined according to ASTM E18. The alloy preferably has intermediate ductility with an elongation less than about 47% as determined according to ASTM E8, and more preferably less than about 43% as determined according to ASTM E8.

The alloy preferably has microstructure that comprises alpha phase, and non-alpha phases in an amount such that the elongation is greater than about 8% as determined according to ASTM E8.

In some embodiments the alloy microstructure preferably comprises at least about 3 volume percent non-alpha phases. In other embodiments alloy microstructure comprises a majority of alpha phase, with between about 3% and about 45% non-alpha phases, and more preferably between about 5% and about 30% non-alpha phase.

The composition and the microstructure are preferably such that the chips resulting from the machining of the alloy break readily into smaller pieces conducive to high speed machining.

Further areas of applicability will become apparent from the description provided herein. The description and specific examples in this summary are intended for purposes of illustration only and are not intended to limit the scope of the present disclosure.

## DRAWINGS

The drawings described herein are for illustrative purposes only of selected embodiments and not all possible implementations, and are not intended to limit the scope of the present disclosure.

FIG. 1 is a copper vs. silicon diagram illustrating the compositions of the preferred embodiment;

FIG. 1A is a copper vs. silicon diagram similar to FIG. 1, illustrating compositions of a further preferred embodiment;

FIG. 2 is a photomicrograph showing an alloy that failed the NSF 14-2012 corrosion requirement;

FIG. 3 is a copper vs. silicon diagram similar to FIG. 1, showing corrosion measurements, made in accordance with ISO 6509;

FIG. 4 is a copper vs. silicon diagram similar to FIG. 1, showing elongation measurements (percentages);

FIG. 5 is a photomicrograph at 1000 $\times$  of Sample S, showing nearly 100% alpha phase;

FIG. 6 is a photomicrograph at 1000 $\times$  of Sample U, showing nearly 100% alpha phase;

FIG. 7 is a photomicrograph at 1000 $\times$  of Sample -8, showing an significant volume of non-alpha phases;

FIG. 8 is a photomicrograph at 1000 $\times$  of Sample O, showing a significant volume of non-alpha phases;

FIG. 9 is a photomicrograph at 1000 $\times$  of Sample M, showing a significant volume of non-alpha phases;

FIG. 10 is a photomicrograph at 1000 $\times$  of Sample N, showing a greater volume of non-alpha phases when compared to Samples -8, O, and M;

FIG. 11 is a photograph of a fitting machined from the samples;

FIG. 12 is a photograph of an additional fitting machined from Sample S;

FIG. 13 is a photograph showing the long, unbroken ribbon chip from machining Sample U;

FIG. 14 is a photomicrograph at 40 $\times$  of the part shown in FIG. 11 made from Sample U, showing an edge burr;

FIG. 15 is a photomicrograph at 50 $\times$  of the part shown in FIG. 12 made from Sample S, showing an edge burr;

FIG. 16 is a photomicrograph at 40 $\times$  of a part shown in FIG. 11 made from Sample U, showing the thread area with alternating shear areas and breakage areas;

FIG. 17 is a photomicrograph at 50 $\times$  of a part shown in FIG. 12 made from Sample S, showing the thread area with alternating shear areas and breakage areas;

FIG. 18 is a photograph of a drill chip from Sample U;

FIG. 19 is a photograph of form tool chips from Sample U;

FIG. 20 is a photograph showing long unbroken ribbon chips from Sample S;

FIG. 21 is a photograph showing a part made from Sample O, showing smooth threads, with a sharp cut;

FIG. 22 is a photograph showing short chips of all three chips shapes from Sample M;

FIG. 23 is a photograph showing short chips of all three chips shapes from Sample O;

FIG. 24 is a photograph showing ribbon chip fragments from Sample B;

FIG. 25 is a photograph of drill chips from Sample B;

FIG. 26 is a photograph of form tool chips from Sample B;

FIG. 27 is a photograph of ribbon and drill chips from Sample -8; and

FIG. 28 is a photograph of form tool chips from Sample -8.

10 Corresponding reference numerals indicate corresponding parts throughout the several views of the drawings.

## DETAILED DESCRIPTION

Example embodiments will now be described more fully with reference to the accompanying drawings.

The composition of a first preferred embodiment of a wrought, machinable, low lead, low copper, silicon, zinc alloy is shown in FIG. 1 as having a copper content of between about 66 weight percent and about 70 weight percent, and a silicon content of between about 1.3 weight percent and about 2.0 weight percent, the balance being primarily zinc with unavoidable impurities, and optional alloying elements as described below.

25 This composition is identified generally as 20 in FIG. 1. The inventors' data indicates that alloys that have copper greater than about 66 weight percent, and silicon greater than about 1.3 weight percent generally are resistant to de-zincification corrosion and consequently pass NSF 14-2012 ISO 6509 requirements, and are preferred. The inventors' data indicates that alloys below about 2 weight percent silicon generally have sufficient ductility to aid mill processing and are preferred. The inventors' data further indicates that alloys above about 1.3 weight percent silicon 30 (and more preferably above about 1.5 weight percent silicon) and below about 70 weight percent copper (and more preferably below about 69 weight percent copper), generally limit ductility sufficiently to machine well, as the resulting chips break into smaller pieces and are preferred.

40 The composition of a second preferred embodiment of a wrought, low lead, low copper, silicon, zinc alloy is shown in FIG. 1A. The composition of FIG. 1A has a copper content of between about 66 weight percent and about 70 weight percent (and more preferably between about 66 weight percent and about 69 weight percent), and a silicon content of between about 1.3 weight percent and about 2.0 weight percent (and more preferably between about 1.5 weight percent and about 2.0 weight percent), the balance being primarily zinc with unavoidable impurities, and optional alloying elements as described below.

45 In addition, the composition of a second preferred embodiment of the alloy is preferably below line 32, given by the equation  $Si=0.167*Cu-9.28$ . The composition of the alloy is preferably above line 34, given by the equation  $Si=0.132*Cu-7.66$ . Thus, the area composition is represented as 30 in FIG. 1A, with between about 66 and about 70 weight percent copper, between about 1.3 weight percent and about 2.0 weight percent silicon, the balance comprising primarily zinc, and unavoidable impurities or specified alloying elements, and the Si content further satisfies the relationship:  $0.167*Cu-9.28 > Si > 0.132*Cu-7.66$ .

50 In alternative embodiments, the copper content is less than about 69 weight percent. In other alternative embodiments the silicon content is greater than 1.5 weight percent.

55 In still other alternative embodiments, the copper content is less than about 69 weight percent and the silicon content is greater than 1.5 weight percent.

TABLE 1

| Example Compositions             |       |      |       |       |        |        |       |        |
|----------------------------------|-------|------|-------|-------|--------|--------|-------|--------|
| Table 1 - Compositions Evaluated |       |      |       |       |        |        |       |        |
| ID                               | Cu    | Si   | Pb    | Fe    | Sn     | Ni     | P     | Zn     |
| (K)                              | 73.5  | 2.79 | 0.079 | 0.043 | 0.012  | 0.004  | 0.084 | 23.44  |
| LCE2                             | 73.05 | 2.48 | 0.04  | 0.045 | —      | 0.004  | 0.093 | 24.29  |
| LCE1                             | 72.57 | 2.45 | 0.04  | 0.046 | 0.004  | 0.004  | 0.091 | 24.8   |
| (J)                              | 71.6  | 1.68 | 0.104 | 0.043 | 0.02   | 0.007  | 0.059 | 26.48  |
| (B)                              | 69.56 | 1.57 | 0.089 | 0.044 | 0.018  | 0.006  | 0.063 | 28.64  |
| -8                               | 68.8  | 1.47 | 0.106 | 0.037 | 0.039  | 0.006  | 0.068 | 29.47  |
| -7                               | 66.53 | 1.1  | 0.117 | 0.033 | 0.037  | 0.007  | 0.063 | 32.1   |
| (R)                              | 70.32 | 1.23 | 0.084 | 0.049 | 0.034  | 0.007  | 0.072 | 28.19  |
| (S)                              | 70.18 | 0.78 | 0.084 | 0.05  | 0.048  | 0.007  | 0.07  | 28.76  |
| (U)                              | 75.51 | 1.84 | 0.073 | 0.042 | 0.038  | 0.006  | 0.074 | 22.41  |
| (M)                              | 65.46 | 1.55 | 0.094 | 0.048 | 0.017  | 0.005  | 0.067 | 32.76  |
| (N)                              | 68.71 | 2.17 | 0.083 | 0.043 | 0.013  | 0.005  | 0.073 | 28.89  |
| (O)                              | 67.96 | 1.8  | 0.094 | 0.047 | 0.015  | 0.005  | 0.073 | 30     |
| Brittle                          | 66.64 | 2.7  | 0.076 | —     | —      | 0.072  | —     | ~30.50 |
| (QE)                             | 67.52 | 0.89 | 0.095 | 0.068 | 0.071  | 0.011  | 0.032 | 31.3   |
| (NQW)                            | 68.61 | 1.45 | 0.044 | 0.03  | 0.014  | 0.002  | 0.015 | 29.82  |
| (NQE)                            | 68.46 | 1.59 | 0.033 | 0.027 | <0.01  | 0.001  | 0.013 | 28.85  |
| (6H)                             | 68.74 | 1.77 | 0.056 | 0.033 | 0.016  | 0.002  | 0.113 | 29.26  |
| (1S)                             | 69.45 | 1.8  | 0.061 | 0.037 | 0.025  | 0.004  | 0.095 | 28.52  |
| (P2)                             | 67.09 | 1.9  | 0.058 | 0.028 | 0.01   | 0.002  | 0.091 | 30.8   |
| (1P)                             | 66.34 | 1.62 | 0.05  | 0.036 | <0.010 | 0.002  | 0.076 | 31.85  |
| (2P)                             | 67.13 | 1.61 | 0.032 | 0.03  | <0.010 | 0.001  | 0.077 | 31.09  |
| (3B)                             | 68.26 | 1.87 | 0.04  | 0.033 | <0.010 | <0.001 | 0.09  | 29.69  |
| (4B)                             | 68.53 | 1.87 | 0.04  | 0.033 | <0.010 | <0.001 | 0.09  | 29.42  |
| (5B)                             | 69.59 | 2.08 | 0.023 | 0.026 | <0.010 | <0.001 | 0.117 | 28.14  |
| (6B)                             | 69.53 | 2.1  | 0.023 | 0.027 | <0.010 | <0.001 | 0.117 | 28.18  |
| (NP)                             | 70.33 | 1.69 | 0.031 | 0.027 | <0.01  | 0.001  | 0.012 | 27.88  |
| (M1S)                            | 69.66 | 1.61 | 0.22  | 0.03  | 0.01   | 0.001  | 0.012 | 28.32  |
| (M2S)                            | 69.85 | 1.6  | 0.03  | 0.3   | 0.01   | 0.001  | 0.022 | 28.18  |
| (M3S)                            | 71.55 | 1.57 | 0.03  | 0.03  | 0.39   | 0.001  | 0.016 | 26.39  |
| (M4S)                            | 69.74 | 1.63 | 0.06  | 0.06  | 0.01   | 0.002  | 0.014 | 28.31  |
| (M5S)                            | 68.69 | 1.64 | 0.03  | 0.03  | 0.02   | 0.001  | 0.013 | 28.74  |
| (M6S)                            | 69.97 | 1.54 | 0.01  | 0.05  | 0.01   | 0.012  | 0.013 | 28.09  |

Notes

M1S - Al 0.014%, As 0.120%

M4S - As 0.115%, Co 0.099%, Mn 0.089%

M5S - Al 0.825%,

M6S - As 0.005%, Bi 0.133%, Mn 0.031%, Sb 0.093%, Se 0.004%, Te 0.034%

## Corrosion Properties

Corrosion testing was performed to determine conformance to NSF 14-2012 requirements of a maximum depth of penetration to be less than 200  $\mu\text{m}$  on testing per the ISO 6509 protocol. The results are summarized in Table 2.

TABLE 2

| Corrosion Properties |       |      |       |                  |                   |                  |                   |
|----------------------|-------|------|-------|------------------|-------------------|------------------|-------------------|
| ID                   | Cu    | Si   | P     | Max. Depth Long. | Max. Depth Trans. | Avg. Depth Long. | Avg. Depth Trans. |
| (K)                  | 73.5  | 2.79 | 0.084 | 30               | 40                | 10               | 20                |
| LCE2                 | 73.05 | 2.48 | 0.093 | 20               | 20                | 20               | <10               |
| LCE1                 | 72.57 | 2.45 | 0.091 | 40               | 40                | 20               | 10                |
| (J)                  | 71.6  | 1.68 | 0.059 | 30               | 0                 | <10              | 0                 |
| (B)                  | 69.56 | 1.57 | 0.063 | 40               | 0                 | 10               | 0                 |
| -8                   | 68.8  | 1.47 | 0.068 | 30               | 20                | 20               | 10                |
| -7                   | 66.53 | 1.1  | 0.063 | 300              | 60                | 70               | 20                |
| (R)                  | 70.32 | 1.23 | 0.072 | 0                | 0                 | 0                | 0                 |
| (S)                  | 70.18 | 0.78 | 0.07  | 0                | 0                 | 0                | 0                 |
| (U)                  | 75.51 | 1.84 | 0.074 | 0                | 0                 | 0                | 0                 |
| (M)                  | 65.46 | 1.55 | 0.067 | 280              | 170               | 180              | 80                |
| (N)                  | 68.71 | 2.17 | 0.073 | 40               | 40                | 20               | 20                |
| (O)                  | 67.96 | 1.8  | 0.073 | 50               | 40                | 20               | 10                |
| Brittle              | 66.64 | 2.7  | 0.072 | —                | —                 | —                | —                 |
| (QE)                 | 67.52 | 0.89 | 0.032 | 220              | 20                | 30               | <10               |
| (NQW)                | 68.61 | 1.45 | 0.015 | 150              | 60                | 30               | <10               |
| (NQE)                | 68.46 | 1.59 | 0.013 | 70               | 40                | 10               | 10                |
| (6H)                 | 68.74 | 1.77 | 0.113 | 40               | 30                | 20               | 10                |
| (1S)                 | 69.45 | 1.8  | 0.095 | 50               | 30                | 20               | <10               |

TABLE 2-continued

| Corrosion Properties |       |      |       |                  |                   |                  |                   |
|----------------------|-------|------|-------|------------------|-------------------|------------------|-------------------|
| ID                   | Cu    | Si   | P     | Max. Depth Long. | Max. Depth Trans. | Avg. Depth Long. | Avg. Depth Trans. |
| (P2)                 | 67.09 | 1.9  | 0.091 | 70               | 60                | 40               | 30                |
| (1P)                 | 66.34 | 1.62 | 0.076 | 160              | 80                | 110              | 40                |
| (2P)                 | 67.13 | 1.61 | 0.077 | 140              | 60                | 60               | 20                |
| 10 (3B)              | 68.26 | 1.87 | 0.09  | 40               | 30                | 20               | 10                |
| (4B)                 | 68.53 | 1.87 | 0.09  | 20               | 30                | 10               | 10                |
| (5B)                 | 69.59 | 2.08 | 0.022 | 30               | 20                | 20               | 10                |
| (6B)                 | 69.53 | 2.1  | 0.025 | 0                | 0                 | 0                | 0                 |
| (NP)                 | 70.33 | 1.69 | 0.031 | 0                | 0                 | 0                | 0                 |
| (M1S)                | 69.66 | 1.61 | 0.022 | 0                | 0                 | 0                | 0                 |
| (M2S)                | 69.85 | 1.6  | 0.016 | 0                | 0                 | 0                | 0                 |
| (M3S)                | 71.55 | 1.57 | 0.016 | 0                | 0                 | 0                | 0                 |
| (M4S)                | 69.74 | 1.63 | 0.014 | 0                | 0                 | 0                | 0                 |
| (M5S)                | 68.69 | 1.64 | 0.013 | 0                | 0                 | 0                | 0                 |
| (M6S)                | 69.97 | 1.54 | 0.013 | 0                | 0                 | 0                | 0                 |

Notes

M1S - Al 0.014%, As 0.120%

M4S - As 0.115%, Co 0.099%, Mn 0.089%

M5S - Al 0.825%,

M6S - As 0.005%, Bi 0.133%, Mn 0.031%, Sb 0.093%, Se 0.004%, Te 0.034%

Previous testing and literature have indicated that Alloy C27450 routinely fails the corrosion requirement of NSF 14-2012 due to de-zincification. In contrast, alloys C69300 and C26000 routinely pass the NSF 14-2012 requirements. Samples -7 and M, failed the NSF 14-2012 corrosion resistance requirement. Maximum penetration depths of 300  $\mu\text{m}$  and 280  $\mu\text{m}$  were obtained on samples -7 and M, respectively, in excess of the 200  $\mu\text{m}$  maximum. In these samples, penetration was greatest along the pathways of the non-alpha phases present which were in the form of longitudinal stringers, aligned with the extrusion direction. A photograph illustrating this for sample M is shown in FIG. 2. The microstructures of samples -7 and M consisted of multiple phases. These two samples had the highest zinc content at 32.1% and 32.7% for -7 and M, respectively.

35 Samples 1P and NQW and others passed the NSF 14-2012 ISO 6509 requirement. Maximum penetration depths of 160  $\mu\text{m}$  and 150  $\mu\text{m}$  were obtained on samples 1P and NQW, respectively. The compositions of these samples were: 66.34 weight percent Cu, 1.62 weight percent Si, and 31.85 weight percent Zn; and 68.61 weight percent Cu, 1.45 weight percent Si, and 29.82 weight percent Zn, respectively. The chemical differences, both within the base alloys and within the phases present are believed responsible for the performance difference between alloys -7 and M (which failed) and alloys 1P and NQW (which passed). From this data, a corrosion pass-fail boundary can be determined.

55 The compositional boundary lines of: 66% minimum copper coupled with 1.3% minimum silicon content appears to represent a boundary to reliably pass NSF 14-2012 ISO 6509 corrosion testing. All other samples tested within the targeted compositional box passed the NSF 14-2012 requirements of the ISO 6509 test with most having penetration depths  $\leq 100 \mu\text{m}$ . Each of these other samples had lower zinc contents, with the highest being at 31.85 weight percent.

60 ISO 6509 corrosion data for the maximum depth of penetration in the longitudinal direction is summarized in FIG. 3. In summary, the samples passing corrosion criteria had either: a) a single phase microstructure, or b) multi-

phase microstructures with copper contents greater than 66% and silicon contents above 1.3%.

Corrosion data in Table 2 indicates that alloys with copper content below 70 weight percent can pass NSF 14-2012 requirements of the ISO 6509 tests. The preferred compositional range including silicon in the alloy passes the NSF 14-2012 ISO 6509 testing requirements, whereas compositions near but outside this range do not.

#### Mechanical Properties

The tensile strength, yield strength, elongation to fracture, and Rockwell B hardness for various compositions were measured and the results are presented in Table 3.

volume fraction of non-alpha phase(s). The sample composition indicated as "Brittle" broke during the cooling of the cast log and was not processed into finished rod. Generally alloys with Cu<70 weight percent and Si>2 weight percent, and more specifically alloys with Si>0.167\*Cu-9.28, will be brittle or have inadequate ductility for some applications and are thus generally less desirable.

The ductility of the compositions varied, generally with increasing ductility if copper is increased and silicon decreased, and correspondingly decreasing ductility if copper is decreased and silicon increased. This is indicated in FIG. 4. These ductility trends appeared to match metallo-

TABLE 3

| ID      | Cu    | Si   | P     | Strength, ksi |       | Elongation | Hardness, Rockwell | 3/4 |         |        | 1/2    |        |
|---------|-------|------|-------|---------------|-------|------------|--------------------|-----|---------|--------|--------|--------|
|         |       |      |       | Tensile       | Yield |            |                    | B   | Surface | radius | radius | Center |
| (K)     | 73.5  | 2.79 | 0.084 | 77.24         | 40.28 | 20.8       | 81                 | 85  | 84      | 84     |        |        |
| LCE2    | 73.05 | 2.48 | 0.093 | 76.6          | 34.8  | 39.4       | 69                 | 72  | 72      | 71     |        |        |
| LCE1    | 72.57 | 2.45 | 0.091 | 76.7          | 34.7  | 42.7       | 69                 | 71  | 71      | 70     |        |        |
| (J)     | 71.6  | 1.68 | 0.059 | 66.18         | 36.21 | 56         | 74                 | 75  | 70      | 64     |        |        |
| (B)     | 69.56 | 1.57 | 0.063 | 73.43         | 46.24 | 35.2       | 80                 | 83  | 78      | 76     |        |        |
| -8      | 68.8  | 1.47 | 0.068 | 73.04         | 50.42 | 31.9       | 74                 | 80  | 77      | 75     |        |        |
| -7      | 66.53 | 1.1  | 0.063 | 73.21         | 49.68 | 35.9       | 74                 | 79  | 76      | 74     |        |        |
| (R)     | 70.32 | 1.23 | 0.072 | 68.94         | 40.57 | 50.7       | 76                 | 78  | 73      | 70     |        |        |
| (S)     | 70.18 | 0.78 | 0.07  | 63.04         | 40.54 | 47.9       | 66                 | 70  | 66      | 64     |        |        |
| (U)     | 75.51 | 1.84 | 0.074 | 66.28         | 38.79 | 59         | 72                 | 76  | 70      | 62     |        |        |
| (M)     | 65.46 | 1.55 | 0.067 | 81.85         | 55.04 | 12.5       | 86                 | 89  | 86      | 84     |        |        |
| (N)     | 68.71 | 2.17 | 0.073 | 78.76         | 53.8  | 7.1        | 86                 | 90  | 86      | 83     |        |        |
| (O)     | 67.96 | 1.8  | 0.073 | 78.12         | 53.14 | 19.6       | 82                 | 87  | 84      | 82     |        |        |
| Brittle | 66.64 | 2.7  | 0.072 |               |       |            |                    |     |         |        |        |        |
| (QE)    | 67.52 | 0.89 | 0.032 | 67.8          | 47.36 | 40.3       | 72                 | 76  | 72      | 66     |        |        |
| (NQW)   | 68.61 | 1.45 | 0.015 | 73.47         | 50.94 | 35.7       | 79                 | 83  | 79      | 77     |        |        |
| (NQE)   | 68.46 | 1.59 | 0.013 | 73.14         | 50.68 | 34.9       | 78                 | 82  | 78      | 67     |        |        |
| (6H)    | 68.74 | 1.77 | 0.113 | 73.64         | 51.05 | 27.7       | 78                 | 82  | 79      | 70     |        |        |
| (1S)    | 69.45 | 1.8  | 0.095 |               |       |            |                    | 81  | 84      | 82     | 77     |        |
| (P2)    | 67.09 | 1.9  | 0.091 | 79.39         | 55.57 | 10.2       | 85                 | 91  | 87      | 85     |        |        |
| (1P)    | 66.34 | 1.62 | 0.076 | 77.33         | 53.06 | 19.1       | 73                 | 87  | 84      | 81     |        |        |
| (2P)    | 67.13 | 1.61 | 0.077 | 73.3          | 52.41 | 22.4       | 67                 | 87  | 80      | 81     |        |        |
| (3B)    | 68.26 | 1.87 | 0.09  | 74.61         | 53.5  | 19.4       | 71                 | 85  | 85      | 76     |        |        |
| (4B)    | 68.53 | 1.87 | 0.09  | 72.17         | 50.95 | 31         | 65                 | 82  | 79      | 82     |        |        |
| (5B)    | 69.59 | 2.08 | 0.117 | 73.99         | 51.27 | 29.7       | 68                 | 84  | 80      | 77     |        |        |
| (6B)    | 69.53 | 2.1  | 0.117 | 76.7          | 53.66 | 20.1       | 74                 | 86  | 86      | 78     |        |        |
| (NP)    | 70.33 | 1.69 | 0.012 | 71.85         | 49.08 | 35.7       | 75                 | 78  | 75      | 64     |        |        |
| (M1S)   | 69.66 | 1.61 | 0.012 | 74.55         | 48.98 | 36.1       | 75                 | 82  | 80      | 75     |        |        |
| (M2S)   | 69.85 | 1.6  | 0.022 | 76.75         | 49.71 | 36.4       | 77                 | 83  | 80      | 73     |        |        |
| (M3S)   | 71.55 | 1.57 | 0.016 | 67.78         | 41.07 | 32.8       | 72                 | 78  | 71      | 56     |        |        |
| (M4S)   | 69.74 | 1.63 | 0.014 | 73.74         | 47.11 | 35.5       | 78                 | 82  | 79      | 57     |        |        |
| (M5S)   | 68.69 | 1.64 | 0.013 | 82.41         | 55.44 | 14.9       | 84                 | 88  | 86      | 83     |        |        |
| (M6S)   | 69.97 | 1.54 | 0.013 | 67.01         | 41.73 | 38.6       | 74                 | 75  | 69      | 54     |        |        |

## Notes

M1S - Al 0.014%, As 0.120%

M4S - As 0.115%, Co 0.099%, Mn 0.089%

M5S - Al 0.825%

M6S - As 0.005%, Bi 0.133%, Mn 0.031%, Sb 0.093%, Se 0.004%, Te 0.034%

The percentage elongation to fracture obtained via tensile testing varied significantly among samples. Sample U broke after 59% elongation, (a high value indicating very ductile material that stretches well but is difficult to fracture). It, along with similar samples, (S) having very high elongation values had a microstructure composed of either all alpha phase, or only having minimal trace percentages of other phases.

In contrast, sample O, a sample with similar silicon percentage as sample U, broke after 19.6% elongation, (a lower value or less ductility). Sample O, although it has a similar silicon percentage to sample U, has less copper and more zinc.

Metallographically, the microstructure of this sample (with 5.5% less copper than U) had a significantly large

graphic versus composition trends in unison with the percentage of non-alpha phases visible in the microstructure.

#### Microstructure

The microstructures presented in the Figures represent a "wrought" condition obtained by subsequent working and heating of a cast product. It is believed that the microstructure and properties of wrought material differ from those of an "as-cast" product with the same composition.

Representative selected micrographs of longitudinal sections at 1,000 $\times$  are shown in FIGS. 5-10. Samples for property testing of: corrosion, mechanical, machining, and microstructure are from wrought mill finished rod that was: cast, hot worked, and then cold drawn to finish dimensions. The area reduction from working was preferably at least 4:1 and more preferably at least 5:1

Twinned alpha ( $\alpha$ ) grains are the primary phase in all samples evaluated. The volume fraction of this phase varied from 60-100%, and varied with composition. Alpha phase is a face-centered-cubic (fcc) microstructure that is very ductile. In samples with higher percentages of zinc and/or silicon, longitudinal stringers of non-alpha phase(s) are also present. These phases generally have less cold ductility when compared to alpha phase.

FIGS. 5-6 show compositions with a structure having a low volume fraction of non-alpha phases present. Casting dendrites and the associated micro-segregation and chemical coring are not readily apparent. It is believed this is a result of the processing after casting that was performed. Alloys of this type machined with difficulties as long ribbon chips were encountered. The ribbons, when difficult to fracture, formed tangled "hair balls" which did not discharge from the machine uniformly. This generated chip interference issues leading to observed chatter on parts and other machine operation difficulties. These compositions, represented samples by S and U, are identified as Group L.

FIGS. 7, 8, and 9 show compositions with a structure having a significant volume fraction of non-alpha phases present. This microstructure was observed with alloys with  $\text{Si} > 1.3$  weight percent. These alloys machined well with short chips. These compositions, represented by samples -8, M, and O, are identified as Group S.

Sample N at 2.17 weight percent silicon was the lowest elongation material finished into parts. Although this composition machined well with small chips, the parts were fragile and split in a "brittle" manner after being deformed. Additionally, some mill processing issues were encountered during the processing of this lower elongation material. Due to these issues, the preferred alloy contains less than 2.0 weight percent silicon consistent with obtaining a desired set of properties. The microstructure of sample N is shown in FIG. 10.

#### Chip Size

FIGS. 13, 18-20, and 22-28 show the machining swarf (chips) obtained during the machining of various compositions of alloys into a fitting for a water hose shown in FIG. 11. In excess of 100 parts were successfully machined from each composition from octagonal cross-section shape with a dimension of 1.062" across (flat-to-flat), using a six spindle Acme screw machine. The machine used has a history of running this part out of leaded brass and lead-free brass alloys. Run speed was at a typical production part rate of 1 part per 2.5 seconds. Machining was monitored for: chip size and breakage characteristics, part smoothness of finish, part dimensions, temperature rise of cutting fluid, and machine torque load. Of these the most informative was the chip length and breakage characteristics as pronounced differences among compositions were detected.

Tooling geometries and machining speeds were not altered during these trials. Therefore, neither a determination of optimal machining conditions nor a precise "machinability rating" value for each of these compositions was made. Instead a boundary between poor and unacceptable versus acceptable was determined.

Samples of the machining swarf (chips) were taken at the discharge conveyor of the machine. The machining processes generated three major chip types, each at roughly 0.020" thick. These are (1) a slender ribbon approximately 0.020" thick  $\times$  0.040"  $\times$  length (Ribbon Chip); (2) a spiral chip from an inside diameter hole approximately 0.020"  $\times$  0.350"  $\times$  length (Drill Chip); and (3) an irregularly shaped chip with fingerlike projections off of a side band generated from an outside form tool. Dimensions were roughly 0.020" thick  $\times$

0.020" with 0.350" long fingers  $\times$  length (Form Chip). Of these the ribbon chip (#1) swarf is considered to most clearly indicate differences in machining performance.

#### Alloy Machining Behavior

Two groupings of chip behavior were noted during evaluation. There are compositions that produced long ribbon chips that were difficult to fracture. This group encountered machining difficulties or concerns. This machining group aligns with Group L, microstructure group with a low fraction of non-alpha phases, detailed previously. Compositions that machined without issue, aligned with Group S. For compositions that measured higher elongation on tensile testing, the discard chips were in general longer, especially the ribbon chip.

The highest elongation sample U, had the slender ribbon chip form into tangled "hair balls" that were difficult to fracture by hand bending. These tangles did not always drop out of the bottom of the screw machine and discharge properly. These chips are shown in FIG. 13. Consequently, the machine had to be stopped and cleaned of scrap several times before machining was able to resume for additional parts. The ribbon chips formed remained relatively ductile and did not readily fracture upon being bent 90°. An unacceptable burr remained along the octagon edge on some parts from this grouping. This is shown in FIG. 14 (for Sample U) and FIG. 15 (for Sample S). Additionally, several parts had periodic chatter marks on the threaded area that may be related to interference issues with ribbon tangles. This is shown in FIG. 16 (for Sample U) and FIG. 17 (for Sample S). This undesirable irregular thread finish was not noted in Group S.

During machining of Group L compositions, chip types referred to as the form and drill initially had some long chips exiting the machine. However, as multiple parts were produced, the chips were generally shorter. It is believed this is likely due to the additional bending the chips and scrap was forced to do because of the interference generated from the ribbon chips. Drill chips from sample U were generally long and unbroken and are shown in FIG. 18. Form tool chips from Sample U are shown in FIG. 19.

Sample S had similar chips to sample U but machining stoppages were not encountered during the limited number of parts produced. Ribbon chips from sample S are shown in FIG. 20.

No machining difficulties were encountered on compositions from Group S and the part finish was deemed to be excellent. Threads were smooth and sharp. FIG. 21 is a photograph of threads from sample O. In contrast to Group L, Group S samples, with lower elongation values on the tensile test had all the chip types fracture into small pieces prior to exiting the machine. The microstructure of Group S had a significant volume of non-alpha phase(s) present. Chips that were collected and photographed are an assortment of fragments of all three chip forms.

Samples M, O, B, and -8 had small and/or readily breakable chips and are shown in FIGS. 22-28, respectively. FIG. 22 shows Sample M. FIG. 23 shows Sample O. Sample M did not pass the corrosion requirement of NSF 14-2012 whereas O was acceptable. Sample O both processed and machined well. FIGS. 24 through 28 are photographs of chips from samples: B (FIGS. 24-26), and -8 (FIGS. 27-28).

#### Other Alloying Elements

##### Lead

Lead does not form a solid solution in the matrix of Cu-Zn-Si alloys, but instead disperses to improve machinability, while silicon typically improves machinability by producing non-alpha phases in the structure of metal.

Lead can optionally be added to improve machinability, preferably in amounts of at least 0.005 weight percent, and more preferably in amount of at least 0.02 weight percent. The addition of lead in an amount exceeding 0.5 weight percent can have an adverse effect, resulting in a rough surface condition, poor hot workability such as poor forging behavior, and low cold ductility. Moreover, maintaining the lead content below 0.5 weight percent complies with many of the lead-related regulations. More stringent regulations have a limit of 0.25 weight percent and some lower than 0.1 weight percent.

#### Antimony and Arsenic

Antimony and arsenic in small quantities can be effective in improving the dezincification corrosion resistance and other properties. Preferably these elements are present in amounts of at least 0.02 weight percent. However, the addition of antimony and/or arsenic in excess of 0.15 weight percent does not produce results in proportion to the excess quantity added. Rather, it can negatively affect the hot forgeability and extrudability.

#### Phosphorus

Phosphorus is similar to antimony and arsenic in that small quantities can be effective in improving dezincification corrosion resistance and other properties. Phosphorus is preferred in some applications to antimony and arsenic due to potential toxicity concerns. Preferably phosphorous is present in amounts of at least 0.02 weight percent. However, the addition of phosphorus in excess of 0.15 percent by weight does not produce results in proportion to the excess quantity added. Rather, it can negatively affect the hot forgeability and extrudability.

#### Tin

Tin is effective in facilitating the formation of non-alpha phases and works like silicon to improve the machinability of Cu—Zn—Si alloys. Thus, tin when present, can further improve machinability of Cu—Zn—Si alloys. Tin can also improve corrosion resistance, especially against erosion corrosion, dezincification corrosion, and copper leachability. Generally, if present, the tin content should be at least about 0.1 weight percent in order to achieve positive effects against corrosion. However, when tin content exceeds 1.2 weight percent, excess tin can reduce ductility of the alloy, so cracks occur more easily when cast. Thus, tin content is preferably less than 1.2 weight percent, and more preferably between 0.2 and 0.8 weight percent.

#### Aluminum

Aluminum is effective in facilitating the formation of non-alpha phases and works like silicon to improve the machinability of Cu—Zn—Si alloys. Aluminum can also be effective in improving the strength, wear resistance, and high-temperature oxidation resistance as well as the machinability of a Cu—Zn—Si alloy. Aluminum also helps keep down the specific gravity of the alloy. Generally, aluminum additions in excess of about 2.5 percent by weight do not produce proportional results. Furthermore, aluminum in excess of 2.5 percent by weight can lower the ductility of the metal alloy without contributing further to the machinability. Additionally, aluminum can decrease the corrosion resistance. For example, sample M5S with 0.825% aluminum had a longitudinal depth of penetration of 800  $\mu\text{m}$  on the ISO6509 test. Due to corrosion concerns, when aluminum is present in excess of 0.5%, the copper content is preferably maintained above 69%.

In some embodiments there may be up to about 1.2 weight percent tin, and preferably up to about 0.8 weight percent tin, and less than about 0.8 weight percent tin, and less than 0.1 weight percent aluminum. In some embodiments there is

up to about 2.5 weight percent aluminum and less than 0.1 weight percent tin. In still other embodiments there is less than about 0.1 weight percent of both tin and aluminum.

#### Bismuth, Tellurium, and Selenium

Bismuth, tellurium, and selenium, like lead, do not form a solid solution with the matrix but disperse to enhance machinability. Thus, one or more of bismuth, tellurium, and selenium can be added to improve machinability. Generally additions of bismuth, tellurium, or selenium in an amount of less than 0.02 percent by weight do not show significant effect on machinability. However, these elements are expensive (compared with copper) and additions in excess of 0.4 percent by weight generally do not pay off economically. Furthermore, with additions of more than 0.4 percent by weight, the alloy can deteriorate in hot workability such as forgeability and cold workability such as ductility. Generally, if present, it is desired to keep the combined content of bismuth, tellurium, or selenium to not higher than about 0.4 percent by weight, to avoid deterioration in hot workability and cold ductility.

#### Nickel, Manganese, Iron, and Cobalt

Nickel, manganese, iron, and cobalt are known to form second phase intermetallic compounds which remove silicon from solid solution. Silicon is important to providing improved stress corrosion cracking resistance as well as good machinability. Iron up to at least about 0.5 weight percent, and nickel, manganese, and cobalt up to at least about 0.25 weight percent each have not been found to have an adverse effect on alloy performance, and allow the use of a varied scrap stream in commercially making the alloy. However is it preferred to keep the manganese and cobalt less than 0.1 weight percent. If present, these elements can provide grain refinement. Above these amounts increased tool wear can be experienced in some types of machining operations.

#### Sulfur

Sulfur can be present up to at least about 0.6 weight percent, but is preferably no more than about 0.25 weight percent.

#### Zirconium and Other Grain Refiners

These results can be achieved without the need for casting grain refining additions, such as zirconium and boron, which are required in other alloys, although in appropriate cases such grain refiners can be used.

The foregoing description of the embodiments has been provided for purposes of illustration and description. It is not intended to be exhaustive or to limit the disclosure. Individual elements or features of a particular embodiment are generally not limited to that particular embodiment, but, where applicable, are interchangeable and can be used in a selected embodiment, even if not specifically shown or described. The same may also be varied in many ways. Such variations are not to be regarded as a departure from the disclosure, and all such modifications are intended to be included within the scope of the disclosure.

#### What is claimed is:

1. A wrought machinable, dezincification-resistant, low lead, low copper, silicon, zinc alloy consisting of between about 66 weight percent and 69 weight percent copper; greater than 1.53 weight percent and less than 2 weight percent silicon wherein the silicon content further satisfies the equation  $0.167*\text{Cu}-9.28>\text{Si}>0.132*\text{Cu}-7.66$ ; up to about 0.25 weight percent lead; up to about 0.15 weight percent phosphorus; up to about 0.5 weight percent iron; up to about 1.2 weight percent tin; up to about 2.5 weight percent aluminum; up to about 0.25 weight percent nickel; up to about 0.25 weight percent cobalt; up to about 0.15

weight percent arsenic; up to about 0.15 weight percent antimony; up to about 0.25 weight percent bismuth; up to about 0.25 weight percent selenium; up to 0.25 weight percent sulfur; and the balance zinc and unavoidable impurities, wherein the alloy has been worked and heated sufficiently to produce a microstructure with a corrosion penetration  $\leq 200 \mu\text{m}$  tested according to ISO 6509 Protocol.

2. The wrought machinable low lead, low copper, silicon, zinc alloy according to claim 1 wherein the alloy has corrosion penetration  $\leq 100 \mu\text{m}$  tested according to ISO 6509 Protocol.

3. The wrought machinable low lead, low copper, silicon, zinc alloy according to claim 1 wherein the microstructure comprises alpha phase and non-alpha phases in an amount such that the elongation is greater than about 8% and less than about 47% as determined according to ASTM E8.

4. The wrought machinable low lead, low copper, silicon, zinc alloy according to claim 1, wherein the alloy has a microstructure comprising a majority of alpha phase, with between about 3 volume percent and about 45 volume percent non-alpha phase.

5. The wrought machinable low lead, low copper, silicon, zinc alloy according to claim 1, wherein the chips resulting from the machining of the alloy break readily into small pieces conducive to high speed machining.

6. A wrought machinable, dezincification-resistant, low lead, low copper, silicon, zinc alloy consisting of between about 66 weight percent and 69 weight percent copper, greater than 1.53 weight percent and less than 2 weight percent silicon wherein the silicon content further satisfies the equation  $0.167\text{Cu}-9.28\text{Si} > 0.132\text{Cu}-7.66$ ; up to about 0.25 lead; up to about 0.15 weight percent phosphorus; up to about 0.5 weight percent iron; up to about 1.2 weight percent tin; up to about 2.5 weight percent aluminum; and up to about 0.25 weight percent nickel; up to about 0.25 weight percent cobalt; up to about 0.15 weight percent arsenic; up to about 0.15 weight percent antimony; up to about 0.25 weight percent bismuth; up to about 0.25 weight percent selenium; up to 0.25 weight percent sulfur; and the balance zinc and unavoidable impurities; the alloy worked and heated sufficiently to produce a microstructure comprising a majority of alpha phase, with between about 3 volume percent and about 45 volume percent non-alpha phase, such that the elongation is greater than about 8% and less than about 47% as determined according to ASTM E8, and a corrosion penetration  $\leq 200 \mu\text{m}$  tested according to ISO 6509 Protocol.

\* \* \* \* \*